

1

2,953,425

## PRODUCTION OF SHAPED OBJECTS FROM VISCOSE

Kurt Heuer, Oberbruch-Grebbien, Bez. Aachen, Hugo Elling, Grebbien, Bez. Aachen, and Richard Elssner, Randerath, Bez. Aachen, Germany, assignors to American Enka Corporation, Enka, N.C., a corporation of Delaware

No Drawing. Filed Oct. 17, 1955, Ser. No. 541,095

Claims priority, application Germany Nov. 25, 1954

4 Claims. (Cl. 18—54)

2

in which Me represents iron, zinc, chromium, cadmium, tin; X represents alkyl amine, alkanol amine or aryl amine; and An represents chloride, sulphate or nitrate.

The process may be carried out in a particularly advantageous manner by using



15

These compounds are added just prior to the spinning operation in amounts of 0.06—0.4% by weight, and preferably 0.12% by weight. Viscoses having a conventional composition of 7 to 8% of cellulose and 5 to 7% of NaOH, with a gamma value of at least 42, are spun at temperatures of 45—70° C. in spinning baths having the following composition: 40—65 g./l. of  $\text{H}_2\text{SO}_4$ , 160—260 g./l. of  $\text{Na}_2\text{SO}_4$  and 30—50 g./l. of  $\text{ZnSO}_4$ . It is expedient to operate with thread withdrawal speeds of 40—60 m./min. The withdrawal speed may be increased, however, if care is taken with the aid of known means to impart to the spinning bath, at least in the first section of its travel after the spinning nozzle, a velocity which is substantially equal to the thread velocity so that the friction between the thread and the spinning bath is thereby substantially reduced. The length of travel in the bath is to be at least 30 cm. In a second bath, which contains approximately 2—10 g./l. of  $\text{H}_2\text{SO}_4$ , the thread is subjected to a drawing of 80—120%, preferably 95—100%, at temperatures higher than 90° C. The thread may then be deposited onto a bobbin, into a centrifuge or onto a perforated web, as desired.

The threads spun by the process according to the present invention have strength values of 380—400 g./100 den., which may be increased by subsequent drawing to 420—440 g./100 den. The finally drawn threads show a very high degree of shrinkage, namely of more than 8%, and have a low degree of swelling.

In order to indicate still more fully the nature of the present invention, the following examples of typical procedure are set forth, it being understood that this description is presented by way of illustration only, and not as limiting the scope of the invention.

50

### Example 1

Alkali cellulose consisting of linters or wood cellulose is sulphidized for 5 hours with 42% of  $\text{CS}_2$  and the xanthate obtained is dissolved to form a viscose with 7.3% of cellulose and 5.5% of NaOH. The viscose is de-aerated, filtered and finally ripened in the usual manner and is mixed 5 hours before being spun with 0.1% by weight of a compound having the formula

60



The viscose is spun with a gamma value of 45 from a spinneret with 1000 orifices to provide a thread of 1650 den., this taking place in a bath with 49 g./l. of  $\text{H}_2\text{SO}_4$ , 200 g./l. of  $\text{Na}_2\text{SO}_4$  and 39 g./l. of  $\text{ZnSO}_4$ . The thread then travels through a distance of 70 cm. in the spinning bath and is withdrawn by a first roller at 23 m./min. The thread then travels through a second bath with 6 g./l.  $\text{H}_2\text{SO}_4$  at a temperature of 90° C. and is withdrawn by a second roller at 46 m./min.; that is to say, it is stretched by 100%. The thread travels from the second roller onto a bobbin and is collected thereon.

the thread is then rewound, washed, finished and dried. It has the following textile data:

| Strength,<br>g./den. |     | Elongation,<br>percent |     |
|----------------------|-----|------------------------|-----|
| dry                  | wet | dry                    | wet |
| 4.2                  | 2.8 | 14                     | 26  |

*Example 2*

0.15% by weight of



is added to a viscose with 7.3% of cellulose and 5.5% of NaOH about 10 minutes before spinning, whereupon it is spun in a bath containing 55 g./l. of H<sub>2</sub>SO<sub>4</sub>, 170 g./l. of Na<sub>2</sub>SO<sub>4</sub> and 45 g./l. of ZnSO<sub>4</sub>, the withdrawal conditions and the stretching being the same as in Example 1. The washed and finished threads are subjected to a final stretching by 8% and are thereafter dried. They have the following textile data:

| Strength, g./den. |     | Elongation, percent |     |
|-------------------|-----|---------------------|-----|
| dry               | wet | dry                 | wet |
| 4.1               | 2.8 | 10                  | 24  |

*Example 3*

0.1% by weight of



is added to a viscose with 7.3% of cellulose and 6% of NaOH about 1 hour before spinning. It is then spun in a spinning bath which contains 60 g./l. of H<sub>2</sub>SO<sub>4</sub>, 220 g./l. of Na<sub>2</sub>SO<sub>4</sub> and 50 g./l. of ZnSO<sub>4</sub>. The bath has a length of 70 cm. It is operated with a thread withdrawal velocity of 23 m./min. and the thread is stretched by 100% by being withdrawn at a velocity of 46 m./min. in a second dilute acid bath at a temperature of 90° C. From the second roller, the thread runs into a centrifuge operating at 6,000 r.p.m. and is given a twist of 120 turns per meter. The thread is then washed and finished and dried after final stretching of 8%. In this way, there are obtained threads with the following textile data:

| Strength<br>g./den. |     | Elongation<br>percent |     |
|---------------------|-----|-----------------------|-----|
| dry                 | wet | dry                   | wet |
| 4.3                 | 3.0 | 12                    | 23  |

While specific examples of preferred methods and products embodying the present invention have been described above, it will be apparent that many changes and modifications may be made in the methods of procedure and the products without departing from the spirit of the invention. It will therefore be understood that the examples cited and the methods and procedures set forth above are intended to be illustrative only and are not intended to limit the invention.

10 What is claimed is:

1. A process for the production of regenerated cellulose threads from viscose, comprising incorporating into viscose 0.06-0.4% by weight based on the viscose of a complex compound having the formula:



wherein Me is selected from the class consisting of Fe, Zn, Cr, Cd, and Sn; X is selected from the class consisting of alkyl amine, alkanol amine, and aryl amine; and An is selected from the class consisting of Cl, SO<sub>4</sub>, and NO<sub>3</sub>, extruding the viscose containing said complex compound into an aqueous bath having approximately the composition 40-65 g./l. of H<sub>2</sub>SO<sub>4</sub> and 30-50 g./l. of ZnSO<sub>4</sub>, and treating the resulting extruded object in a second hot bath containing approximately 2-10 g./l. of H<sub>2</sub>SO<sub>4</sub> and stretching same by a factor of approximately 80-120%.

2. A process according to claim 1, wherein the complex compound has the formula:



3. A process according to claim 1 wherein the complex compound has the formula:



35 4. A process according to claim 1 wherein the complex compound has the formula:



References Cited in the file of this patent

UNITED STATES PATENTS

|    |           |                |                |
|----|-----------|----------------|----------------|
| 40 | 2,077,412 | Herzog         | Apr. 20, 1937  |
|    | 2,284,028 | Ubbelohde      | May 26, 1942   |
|    | 2,506,249 | Tammen         | May 2, 1950    |
|    | 2,516,316 | Hare           | July 25, 1950  |
|    | 2,535,044 | Cox            | Dec. 26, 1950  |
| 45 | 2,580,473 | Sowa et al.    | Jan. 1, 1952   |
|    | 2,593,466 | Mac Laurin     | Apr. 22, 1952  |
|    | 2,648,611 | Richter        | Aug. 11, 1953  |
|    | 2,664,360 | Charles et al. | Dec. 29, 1953  |
|    | 2,705,184 | Drisch         | Mar. 29, 1955  |
| 50 | 2,732,279 | Tachikawa      | Jan. 24, 1956  |
|    | 2,772,444 | Burrows        | Dec. 4, 1956   |
|    | 2,784,107 | Tallis et al.  | Mar. 5, 1957   |
|    | 2,796,319 | Studer         | June 18, 1957  |
| 55 | 2,852,333 | Cox et al.     | Sept. 16, 1958 |
|    | 2,884,332 | Locher         | Apr. 8, 1959   |
| 60 | 2,892,729 | Howsmon        | June 30, 1959  |